# EUROPEAN PATENT SPECIFICATION

(11) **EP 3 222 913 B1**
(45) Date of publication and mention of the grant of the patent: **26.05.2021**
(21) Application number: 14906429.7
(22) Date of filing: 17.12.2014
(51) Int. Cl.: F23K 1/00, F23K 3/02, F23L 7/00, F23M 5/08, F23G 5/44, F23G 7/02, F23G 7/10, F23J 1/08

(54) **BIOMASS MICRON FUEL HIGH-TEMPERATURE CLEAN COMBUSTION METHOD BASED ON ADIABATIC COMBUSTION CONDITIONS**
HOCHTEMPERATUR-VERBRENNUNGSVERFAHREN ZUR SAUBEREN VERBRENNUNG VON BIOMASSE-MIKRON-BRENNSTOFF AUF DER BASIS VON ADIABATISCHEN VERBRENNUNGSBEDINGUNGEN
PROCÉDÉ DE COMBUSTION NETTE À HAUTE TEMPÉRATURE DE BMF (BIOMASS MICRON FUEL) BASÉ SUR DES CONDITIONS DE COMBUSTION ADIABATIQUE

(30) Priority: 19.11.2014 CN 201410665874
(43) Date of publication of application: 27.09.2017
(73) Proprietor: Huazhong University of Science and Technology, Wuhan, Hubei 430074 (CN)
(72) Inventor: XIAO, Bo, Wuhan Hubei 430074 (CN); HU, Zhiquan, Wuhan Hubei 430074 (CN); LIU, Shiming, Wuhan Hubei 430074 (CN); JIN, Shiping, Wuhan Hubei 430074 (CN); YANG, Jiakuan, Wuhan Hubei 430074 (CN); GUAN, Yanwen, Wuhan Hubei 430074 (CN); SHU, Zhaohui, Wuhan Hubei 430074 (CN); LIU, Wenbin, Wuhan Hubei 430074 (CN)
(74) Representative: Lang, Christian
(86) International application number: PCT/CN2014/094005
(87) International publication number: WO 2016/078176

(56) References cited:
- CN-A- 101 935 568
- CN-B- 101 935 568
- CN-U- 202 379 954
- JP-A- 2005 265 300
- JP-A- 2009 180 476
- JP-A- 2014 202 448
- US-A1- 2009 078 175
- LIU, SHIMING ET AL.: 'An Experimental Study on Air-steam Gasification of Biomass Micron Fuel (BMF)''.' ACTA ENERGIAE SOLARIS SINICA vol. 31, no. 2, 28 February 2010, pages 237 - 240, XP008185370

## Description

The invention belongs to the field of renewable clean energy resource, more particularly, it refers to a method for clean-burning and using micron-size biomass fuel under the adiabatic condition.

Nowadays, the depletion and exhaustion of fossil energy and deterioration of environment have made it urgent to develop renewable and clean energy resource and reuse waste. The biomass fuel refers to the agricultural and forestry residues including straw, saw dust, bagasse, and rice husk, etc. The agricultural and forestry residues are grinded, mixed, squeezed, and dried to form a novel clean fuel which can be directly burnt. The development of biomass fuel can not only wisely use the agricultural and forestry residues to prevent waste of resources, the emissions of carbon dioxide, sulfur dioxide, and nitrogen oxides can also be reduced and haze can be avoided. Therefore, the clean fuel would be applied widely at home and abroad.

JP 2014202448 A discloses a power generation method. The method includes feeding coal and palm seed hull into a crusher and crushing the mixture; supplying the pulverized product to a furnace and combusting to produce steam; and utilizing the steam to generate electricity.

US 20090078175 A1 discloses a fuel flexible furnace. The furnace includes a main combustion zone; a reburn zone downstream from the main combustion zone; and a delivery system operably coupled to supplies of biomass and coal and configured to deliver the biomass and the coal to the main combustion zone and the reburn zone.

JP 2005265300 A discloses a boiler device. The device utilizes various fuels, such as pulverized coal, sludge, biomass fuels. The boiler device includes a furnace, a partial combustion furnace, a fuel nozzle, a heat exchanger, a high-temperature air supply nozzle, an air preheater, and a secondary air supply unit.

The inventor of the application has put forward the patent application CN101935568A about micron-size biomass fuel combustion at 2010. The patent disclosed a biomass fuel formed by combining micron-size plant fiber powers with additives, and in a plurality of tests it is suggested that the combustion temperature of the micron-size biomass fuel is about 1300°C at average (the peak temperature is 1370°C), and the combustion efficiency of the biomass fuel is above 96%, in addition, the harmful components content in the waste gas of combustion can be effectively reduced.

However, follow-up studies revealed that the patent has the following shortcomings and defects: first of all, for most of the industrial applications, such as an efficient boiler steam power-generation system, the combustion temperature of fuel needs to be higher than 1500°C, which is decided by the Carnot cycle principle, only after the boiler fuel reach to a sufficient high combustion temperature, high-temperature and high-pressure steam can be generated, and further utilize the mechanical energy converted for power generation which have the economic value. Meanwhile, some of the high-temperature industrial stoves characterized by the high consumption and high emission also require the combustion temperature to reach above 1500°C, such as refractory materials, cement and glass, etc. However, the combustion temperature using existing micron-size biomass materials burning in a normal way failed to reach that high temperature. In addition, high temperature is one of the most sensitive and important conditions during industrial production. Industrial data shows that every 50°C elevation of combustion temperature can cover more industrial production needs. Moreover, the radiant heat transfer efficiency is proportional to the fourth power of the temperature. For example, when the combustion temperature of fuel increased from 1400°C to 1450°C, the thermal energy obtained by the heating body from the radiant heating is improved by 12%, meanwhile, the rise of combustion temperature further increases the combustion speed and combustion efficiency of the fuel. Under this circumstance, how to further improve and stabilize the combustion temperature and combustion efficiency of the micron-size biomass fuel, so as to broaden the application thereof in industrial environment becomes an urgent technical problem to be solved. Lastly, according to the analysis of the chemical composition, we know that the micron-size biomass fuel is a complex and solid high-molecular hydrocarbon material, and is hard to burn at a rapid rate, since the biomass fuel contains more carbon than hydrogen, the small molecules containing hydrogen burn first and inevitably, tar, residual carbon and ash content in solid state which are difficult to react with oxygen are produced. Meanwhile, the tar, residual carbon, and ash content remain in the combustion chamber of boiler for a while, and once the tar, residual carbon, and ash content do not fully react with the oxygen in time, the tar, residual carbon, and ash content are discharged as waste resources, and further form aerosol and pollutant source of haze to pollute the environment.

In view of the above-described problems, it is one objective of the invention to provide a method for clean-burning micron-size biomass fuel under the adiabatic condition. According to the characteristics of the micron-size biomass fuel and the construction features of the industrial stove, the specific design and researches have been done on the operating procedure, key process parameters, and combustion mechanism of the biomass fuel combustion, the method obtains the combustion temperature as high as 1500°C to satisfy the heating requirements for more industrial high-temperature boilers. Meanwhile, compared with the prior art, the method barely produces tar, residual carbon, or ash content, thus the method is applicable to the clean and high-temperature burning environment in the industrial production.

To achieve the above objective, in accordance with the invention, there provided a method for clean-burning micron-size biomass fuel under the adiabatic condition, comprising:
1) grinding raw biomass material composed of plant fiber to solid powders, which can be served as micron-size biomass fuel. The solid powders have an average particle size smaller than 400 µm; encapsulating the micron-size biomass fuel; loading and transporting the micron-size biomass fuel to industrial stoves for burning via pipelines;
2) premixing the micron-size biomass fuel with air to form flowing dust cloud prior to entering the industrial stoves, and set the excess air coefficient between 0.98 and 1.25 during the operation.
3) ejecting the flowing dust cloud premixed in 2) to an adiabatic combustion chamber in the industrial stoves via a fuel nozzle along a tangential direction, and the adiabatic combustion chamber being a relatively sealed heat storage space comprising a side wall made from an insulating material layer; the volumetric combustion intensity of the adiabatic combustion chamber is set between 150 and 400 kg/m³; surrounding the side wall using a heating body of the industrial stoves, and controlling heat flowing through the side wall to be less than 10% of combustion energy of the micron-size biomass fuel; the fuel nozzle being at least one in number, and the velocity of ejection being between 1 and 10 m/s; gasifying and burning the flowing dust cloud at a distance between 0.5 and 2.5 time(s) the diameter of the fuel nozzle to obtain a combustion temperature between 1500 and 1600°C, the high-temperature flame ejected from the adiabatic combustion chamber to heat the heating body;
4) adding moderate steam to the adiabatic combustion chamber during combustion, and a mass ratio of the micron-size biomass fuel to the steam being 1:30-150 to accelerate gasification and decomposition of intermediates comprising tar and carbon particles produced during the combustion prior to departing from the flame; discharging melted ash content in a form of liquid glass at the bottom part of the adiabatic combustion chamber after the residual ash content melted and separated from the high temperature flame when the combustion is completed.

In a class of this embodiment, in 1), the micron-size biomass fuel comprises more than 35 wt.% of powders having a particle size smaller than 50 µm. The micron-size biomass fuel comprises more than 75 wt.% of powders having a particle size smaller than 100 µm. The micron-size biomass fuel comprises more than 90 wt.% of powders having a particle size smaller than 250 µm.

In a class of this embodiment, in 1), the micron-size biomass fuel is rigidly or flexibly sealed in a container to be loaded and transported, and the volume of the container is between 1.5 and 90 m³.

In a class of this embodiment, in 2), preferably, the excess air coefficient is set between 1.0 and 1.15.

In a class of this embodiment, in 3), preferably, the volumetric combustion intensity of the adiabatic combustion chamber is set between 200 and 300 kg/m³, and the heat flowing through the side wall is no more than 3%-6% of the combustion energy of the micron-size biomass fuel.

In a class of this embodiment, in 3), preferably, the adiabatic combustion chamber is a relatively sealed heat storage space comprising the side wall made from an insulating material layer of alumina fiber, and the thickness of the side wall is between 80 and 320 mm. A height of the adiabatic combustion chamber is between 0.8 and 4 time(s) the diameter of the adiabatic combustion chamber.

In a class of this embodiment, in 4), preferably, the mass ratio of the steam to the micron-size biomass fuel is 1:60-120.

In a class of this embodiment, preferably, the industrial stoves are boilers that served as boiler steam power-generation system, or stoves made from cement, glass, ceramics, etc.

Advantages of the method for clean-burning micron-size biomass fuel under the adiabatic condition according to embodiments of the invention are summarized as follows:
1. The adiabatic combustion chamber is provided, and the key parameters including volumetric combustion intensity and contact temperature are set up according to the combustion of the micron-size biomass fuel to form a relatively sealed heat storage space so that combustion energy of the biomass fuel with a relatively low energy density is accumulated and high-temperature combustion condition is formed in the adiabatic combustion chamber. Meanwhile, the gasification and combustion of the powders are simultaneously and instantly completed in the same space to produce ultra-high temperature combustion, and the high combustion temperature further improves the combustion speed and combustion efficiency of the micron-size biomass fuel, thus the average combustion temperature is obviously increased compared to the combustion temperature in the prior art, and the combustion efficiency is above 98%. The ultra-high temperature combustion of the micron-size biomass fuel not only completely decomposes the intermediates including tar and carbon particles, but also melts the incombustible inorganic components. The melted inorganic component is then discharged from the bottom of the stoves as liquid slag. Therefore, the production of clean-burning of the solid biomass fuel includes no tar, residual carbon, or ash content.
2. The solid biomass fuel is hermetically encapsulated, loaded, and transported, and the transportation of the bulky and flammable micron-size biomass fuel with a relatively low energy density is low-cost, efficient, and safe, thus the method satisfies the requirements of industrial-scale energy supplement and application.
3. The micron-scale biomass fuel is premixed with the air using certain excess air coefficient before the fuel enters the industrial stoves. Tests show that the premixing can effectively increase the possibility of oxygen expanding to the surface of bio-particles in the flowing dust cloud, and ensure the complete combustion of bio-particles. In addition, the premixing, in combination with the adiabatic conditions, improve the temperature peak of the combustion.
4. Specifications and ejection velocity of the adiabatic combustion chamber are specifically designed to ensure that the micron-size biomass fuel have enough residence time and that the components involved in the combustion always float during the combustion process, instead of depositing at the bottom of the combustion chamber, so as to facilitate the sufficient combustion of the fuel and improve the combustion temperature.
5. Steam is added at a certain percentage during the combustion process. Steam served as a gasification agent which can react with the intermediates, and decompose the intermediates to hydrogen and carbon monoxide. Hydrogen accelerates the flame spread rate in the limited combustion space and ensures that the expected temperature peak and combustion efficiency are achieved in a short time.
6. By using the method in the embodiments of the invention, the combustion temperature of the micron-size biomass fuel is further improved to be higher than 1500°C, thus correspondingly satisfying the heating requirements of most of the industrial productions. Especially, the method is applicable to the clean and efficient burning in all kinds of industrial stoves.

FIG. 1 is a flowchart of a method for clean-burning micron-size biomass fuel in accordance with one embodiment of the invention.

FIG. 2 is a diagram showing an application environment of combustion technology comprising an adiabatic combustion chamber in accordance with one embodiment of the invention.

For further illustrating the invention, experiments detailed a method for clean-burning micron-size biomass fuel under the adiabatic condition are described below. It should be noted that the following examples are intended to describe and not to limit the invention. In addition, the technical features mentioned in each example can be combined as long as the features do not conflict with each other.

The combustion temperature of biomass fuel burned using the conventional method at between 700 and 1000°C, thus the biomass fuel can only be applied to household heating and cooking. However, since the industrial revolution, the working temperature is required to be even higher, and the combustion quality is even strictly requested. For example, the reaction temperature of the ceramics is mostly about 1300°C, and the heating temperature from the fuel is required to be above 1500°C; the chemical transition temperature of cement burning is above 1400°C, and the heating temperature from the fuel is required to be above 1500°C to ensure the production efficiency. In an efficient boiler steam power-generation system, the combustion temperature from the fuel is required to be above 1500°C, therefore, the combustion temperature of the biomass fuel directly influence whether the biomass fuel can be applied to modern industry production. On the other hand, when the biomass hydrocarbon fuel burned at a low temperature, incomplete combustion produces tar and residual carbon which further form aerosol and haze. The utilization rate of energy is low, meanwhile, the unburnt hydrocarbon becomes environmental pollutant source, both of which influence the application of biomass fuel in industrial-scale production.

Conventionally, the biomass fuel is burnt using the layer combustion technology, and the fuel failed to fully react with the air in a short period of time in the combustion chamber. The combustion temperature is low, and tar is produced, forming haze. Meanwhile, ash content produced by the layer combustion buries the fuel and hinders the contact and reaction with the oxygen. Certain amount of residual carbon is unburnt and discharged from the combustion chamber as slag, causing waste of resources. Under this circumstance, although burning the micron-size biomass fuel disclosed in the prior patent application can obtain relatively high combustion temperature and effectively reduce pollutant discharge, the combustion temperature of the biomass fuel is limited to be about 1350°C, and actually, tar, carbon particles, and especially ash content residues are not completely avoided, as revealed by follow-up studies. Therefore, a profound study on the combustion process, combustion temperature, combustion efficiency, and the combustion mechanism of the micron-size biomass fuel should be conducted to obtain a higher combustion temperature and to satisfy the heating requirements of industrial high-temperature boilers. Meanwhile, no tar, residual carbon, or ash content is ensured so that the low-cost biomass fuel is applicable to the clean-burning in industrial production.

Specifically, the method for clean-burning micron-size biomass fuel comprises the following steps. The steps are illustrated as follows, and the illustration is mainly focused on the design and principles of the key combustion conditions.

First of all, raw biomass material composed of plant fiber is grinded to solid powders of micron-size biomass fuel, and an average particle size of the solid powders is smaller than 400 µm. The micron-size biomass fuel is hermetically encapsulated, loaded and transported to industrial stoves via pipelines. For example, the biomass fuel is composed of plant fiber and additive. The additive is pulverized coal, pulverized lime, red mud, or a mixture thereof. The plant fiber comprises more than 35 wt.% of powders having a particle size smaller than 50 µm. The plant fiber comprises more than 75 wt.% of powders having a particle size smaller than 100 µm. The plant fiber comprises more than 90 wt.% of powders having a particle size smaller than 250 µm. Similar to the coal, the micron-size biomass fuel is characterized by high consumption and light weight, when the biomass fuel is packaged in bags like the flour, the labor cost is high, and dust flying tends to occur when the bags are opened to discharge the powders, resulting in horrible working environment, waste of resources, and risks of fire outbreak. Meanwhile, the powders in bags are easy to get damp, then the mobility thereof is adversely affected. Once the powders get damp, the cost of drying the powders is higher than the cost of fuel itself. Therefore, in the first step, the micron-size biomass fuel is hermetically encapsulated, loaded and transported to industrial stoves in the form of solid powders, and the transportation of bulky and flammable micron-size biomass fuel with a relatively low energy density is low-cost, efficient, and safe, thus the method satisfies the requirements of industrial-scale energy supply and application.

Then, before the micron-size biomass fuel enters the industrial stoves, the micron-size biomass fuel is premixed with air to form flowing dust cloud, and an excess air coefficient is set between 0.98 and 1.25; preferably, the excess air coefficient is between 1.0 and 1.15. The biomass fuel is premixed using the excess air coefficient to form the flowing dust cloud because firstly the combustion needs air, and especially oxygen in the air. However, in the air, oxygen only accounts for 21%, and the rest of air is the inert gas nitrogen. The molecular weights of oxygen and nitrogen are similar, thus the separation of nitrogen and oxygen is difficult, meanwhile, the oxygen-enriched air and pure oxygen are costly, in reality, fuel is directly burned in the air. When one cubic meter of oxygen enters the adiabatic combustion chamber, four cubic meters of nitrogen enter the adiabatic combustion chamber together with the oxygen, and the nitrogen absorbs heat and decreases the temperature in the combustion chamber, thus in the first place too much air should be avoided from entering in the combustion chamber, and the excess air coefficient is designed to be lower than 1.3. Comparison tests show that when the biomass fuel is at micron-size, without being compressed, the structure of the biomass like a porous network, and oxygen can penetrate into the micropores, in addition, the biomass fuel is rich in volatile components, thus about 70% of the solid structure can be decomposed at 500°C. Meanwhile, due to the high hydrogen content, the excess air coefficient is required to be controlled above 0.98. Practice shows that the excess air coefficient in the invention can effectively improve the possibility of oxygen expanding to the surface of bio-particles in the flowing dust cloud, ensure the complete combustion of bio-particles, reduce the amount of excess air, and increase the combustion efficiency, which means that the excess air coefficient is an important feature which ensures the high-temperature combustion of biomass fuel.

The premixed flowing dust cloud is ejected to the adiabatic combustion chamber in the industrial stoves via a fuel nozzle 11 along a tangential direction. One of the key improvements of the invention is that the adiabatic combustion chamber 1 is a relatively sealed heat storage space comprising a side wall 2 made from an insulating material layer, and a volumetric combustion intensity of the adiabatic combustion chamber is between 150 and 350 kg/m³. The side wall is surrounded by the heating body of the industrial stoves, and heat flowing through the side wall is controlled to be less than 10% of combustion energy of the micron-size biomass fuel. The fuel nozzle is at least one in number, and a velocity of ejection being between 1 and 10 m/s, so that the combustion condition and the combustion speed are controlled. The flowing dust cloud is gasified and floats in the combustion chamber the moment the dust cloud departs from the fuel nozzle, instead of settling at the bottom of the combustion chamber, and the flowing dust is burned instantly (at a distance between 0.5 and 2.5 time(s) the diameter of the fuel nozzle) to obtain a combustion temperature between 1500 and 1600°C at average.

As shown in FIG. 2, the technical results brought by the designs and the principles are specifically explained as follows. Firstly, the adiabatic combustion chamber 1 is provided, and the key parameters including volumetric combustion intensity and contact temperature of the adiabatic combustion chamber are set up according to the combustion of the micron-size biomass fuel to form a relatively sealed heat storage space so that combustion energy of the biomass fuel with a relatively low energy density is accumulated and high-temperature combustion condition in the adiabatic combustion chamber is formed. Meanwhile, the gasification and combustion of the powders are simultaneously and instantly completed in the same space to produce ultra-high temperature combustion, and the high combustion temperature further improves the combustion speed and combustion efficiency of the micron-size biomass fuel, therefore the average combustion temperature is obviously increased compared to that of the prior art, and the combustion efficiency is above 98%. Analyzed from the reaction mechanism, the fuel is not just simply stacked in the combustion chamber, instead, a large amount of fuel molecules collides with oxygen molecules one-to-one, and rapidly release energy in the combustion chamber, which contributes to the accumulation of temperature, and then disappear fast to release space for new fuel coming. In other words, in a unit combustion space and within a unit combustion period, the more heat released from the fuel and accumulated in the space, the higher the combustion temperature is. A great many tests show that the method in accordance with the above design can obtain the combustion temperature as high as between 1500 and 1600°C at average.

In addition, according to the theory of thermal radiation, the radiation force refers to the full wavelength energy emitted by a unit surface area of an object to a hemisphere space per a unit time, and the unit is W/m². The relationship between the radiation force and the temperature is shown as Formula (1): ${E}_{b} = {\int }_{0}^{∞} {E}_{b λ} dλ = {\int }_{0}^{∞} \frac{{c}_{1} {λ}^{- 5}}{{e}^{{c}_{2} / \left(λT\right)}} d λ = {σT}^{4}$

Therefore, when the combustion temperature increased from 1300°C to 1450°C, the radiation force is correspondingly increased: $ρ = \frac{σ \left({1723}^{4}-{1573}^{4}\right)}{σ {1573}^{4}} \times 100 % = 43.95 %$

The tar and residual carbon can be quickly decomposed and burnt in the oxygen at 900°C, and as the combustion temperature in the example of the invention is 1500°C, the tar and residual carbon can be completely decomposed in 0.2 seconds at such a high temperature. Take a 4 t/h industrial boiler as an example, a volume of the adiabatic combustion chamber is 1.8 m³, and the time *τ* that the combustion product remains in the combustion chamber is obtained by: $τ = \frac{V \times 273}{{B}_{j} {V}_{g} \left({t}_{av}+273\right)}$ where, *Bⱼ* is the fuel consumption (kg/s); *V_{g}* is the flue gas volume (Nm³/kg); V is the volume of the combustion chamber (m³); and *tₐᵥ* is the average temperature of the flue gas. The time *τ* that the flue gas remains in the adiabatic combustion chamber is obtained *τ*=0.26 s. Therefore, in the invention, tar and residue carbon can be effectively decomposed at such a high temperature within the residence time of the flue gas. The hydrocarbon is burnt out, and the flue gas exhausted from the combustion chamber contains no tar and carbon particles. A more detailed illustration is made in the following examples.

### Example 1

The feed rate of the micron-size biomass fuel is 700 kg/h; the caloric value of the fuel is 17166 kJ/kg (4100 Kcal/kg); the diameter of an inner chamber of the adiabatic combustion chamber is 1400 mm, and a height of the inner chamber is 1800 mm. The micron-size biomass fuel is premixed with certain amount of air, and is ejected to the combustion chamber from the bottom along a tangential direction at a rate of 5 m/s. The combustion chamber comprises a lining built by firebrick. A thickness of the lining is 114 mm. The lining is coated by alumina fiber cotton for thermal insulation which is highly pure.

Table 1 shows the test results of combustion temperatures varying with different thicknesses of the alumina fiber cotton and with different excess air coefficients:

### Example 2

The feed rate of the micron-size biomass fuel is 705 kg/h; the caloric value of the fuel is 17166 kJ/kg (4100 Kcal/kg); the diameter of an inner chamber of the adiabatic combustion chamber is 1400 mm. The micron-size biomass fuel is premixed with certain amount of air using the excess air coefficient 1.05, and is ejected to the combustion chamber from the bottom along a tangential direction at a rate of 5 m/ s. The combustion chamber comprises a lining built by firebrick. A thickness of the lining is 114 mm. The lining is coated by alumina fiber cotton for thermal insulation which is highly pure, and a thickness of the fiber cotton is 150 mm. Table 2 shows the test results of combustion temperatures varying with different heights of the adiabatic combustion chamber. Table 3 shows the test results of the blackness of flue gas varying with different heights of the combustion chamber and different steam additions.

Because the combustion temperature in the invention has improved 150°C compared to that of the prior art, correspondingly, the radiation force in the combustion chamber is improved by 43%. In addition, the decomposition rate and gasification rate, as calculated above, have also greatly been increased, thus facilitating the clean burning of biomass fuel which barely generates tar, residual carbon, or ash content.

Lastly, steam is added in the adiabatic combustion chamber during combustion, and a mass ratio of the steam to the micron-size biomass fuel is 1:30-150 so as to accelerate gasification and decomposition of intermediates comprising tar and carbon particles produced during the combustion prior to departing from the flame. Melted ash content departs from the flame when the combustion is completed, and is settled at the bottom of adiabatic combustion chamber. The melted ash content in a form of liquid glass is discharged by the slag removal mechanism 4 with a slag removal piston at one side of the inspection manhole 61.

Steam is added because steam as a gasification agent can react with the intermediates during the combustion, and can decompose the intermediates to hydrogen and carbon monoxide. Hydrogen further accelerates the combustion speed and ensures that the expected temperature peak and combustion efficiency are achieved in a short period of time. For example, tests show that the proportion of steam designed in the invention, in combination with other combustion conditions, enables the dust cloud to be completely gasified and burnt at a distance between 0.5 and 2.5 time(s) the diameter of the fuel nozzle after the dust cloud departs from the fuel nozzle.

While particular embodiments of the invention have been shown and described, it will be obvious to those skilled in the art that changes and modifications may be made without departing from the invention in its broader aspects, and therefore, the aim in the appended claims is to cover all such changes and modifications as fall within the scope of the invention as defined in the claims.

## Claims

1. A method for clean-burning micron-size biomass fuel under an adiabatic condition, the method comprising grinding raw biomass material composed of plant fiber to solid powders of micron-size biomass fuel, an average particle size of the solid powders being smaller than 400 µm; and hermetically encapsulating the micron-size biomass fuel; **characterized in that** the method further comprises:
1) premixing the micron-size biomass fuel with air to form a flowing dust cloud having an excess air coefficient between 0.98 and 1.25, prior to entering an industrial stove comprising an adiabatic combustion chamber (1);
2) ejecting the flowing dust cloud premixed in 1) to the adiabatic combustion chamber (1) via a fuel nozzle (11) along a tangential direction , the adiabatic combustion chamber (1) being a sealed heat storage space and the side wall (2) being made from an insulating material layer; setting a volumetric combustion intensity of the adiabatic combustion chamber (1) to be between 150 kg and 350 kg of the biomass fuel per cubic meter of the adiabatic combustion chamber (1); surrounding the side wall using a heating body of the industrial stove, and controlling heat flowing through the side wall (2) to be less than 10% of combustion energy of the micron-size biomass fuel; the fuel nozzle (11) being at least one in number, and a velocity of ejection being between 1 m/s and 10 m/s; completing gasifying and burning of the flowing dust cloud at a distance between 0.5 and 2.5 time(s) the diameter of the fuel nozzle (11) to obtain a combustion temperature between 1500°C and 1600°C; allowing extrusive flame to heat the heating body;and
3) adding steam in the adiabatic combustion chamber (1) during combustion, and a weight ratio of the steam to the micron-size biomass fuel being between 1:30 and 1:150 to accelerate gasification and decomposition of intermediates comprising tar and carbon particles produced during the combustion prior to departing from the flame; discharging melted ash content in a form of liquid glass at a bottom part of the adiabatic combustion chamber (1) after the melted ash content departs from the flame when the combustion is completed.

2. The method of claim 1, **characterized in that** the micron-size biomass fuel comprises more than 35 wt.% of powders having a particle size smaller than 50 µm; the micron-size biomass fuel comprises more than 75 wt.% of powders having a particle size smaller than 100 µm; and the micron-size biomass fuel comprises more than 90 wt.% of powders having a particle size smaller than 250 µm.

3. The method of claim 1, **characterized in that** the micron-size biomass fuel is rigidly or flexibly sealed in a container, and is loaded and transported, and a volume of the container is between 1.5 m³ and 90 m³.

4. The method of claim 1 or 2, **characterized in that** in 1), the excess air coefficient is between 1.0 and 1.15.

5. The method of claim 1, 2, or 3, **characterized in that** in 2), the volumetric combustion intensity of the adiabatic combustion chamber (1) is between 200 kg and 300 kg of the biomass fuel per cubic meter of the adiabatic combustion chamber (1), and the heat flowing through the side wall (2) is no more than 3%-6% of the combustion energy of the micron-size biomass fuel.

6. The method of claim 5, **characterized in that** in 2), the adiabatic combustion chamber (1) is the sealed heat storage space comprising the side wall (2) made from an insulating material layer of inorganic fiber and refractory material, and a thickness of the side wall (2) is between 80 mm and 320 mm; and a height of the adiabatic combustion chamber (1) is between 0.8 and 4 time(s) the diameter of the adiabatic combustion chamber (1).

7. The method of claim 5, **characterized in that** in 3), the weight ratio of the steam to the micron-size biomass fuel is between 1:60 and 1:120.

8. The method of any one of claims 1-7, **characterized in that** the industrial stove is a boiler, or a stove made of cement, glass, or ceramics.

## Patentansprüche

1. Verfahren zum sauberen Verbrennen von mikrometergroßem Biomassebrennstoff unter adiabatischen Bedingungen, wobei das Verfahren das Mahlen von Biomasse-Ausgangsmaterial umfasst, das aus Pflanzenfasern zusammengesetzt ist, zu festen Pulvern aus mikrometergroßem Biomassebrennstoff, wobei die durchschnittliche Partikelgröße der festen Pulver kleiner als 400 µm ist; und das hermetische Verkapseln des mikrometergroßen Biomassebrennstoffs umfasst; **dadurch gekennzeichnet, dass** das Verfahren ferner umfasst:
1) Vormischen des mikrometergroßen Biomassebrennstoffs mit Luft, um eine strömende Staubwolke zu bilden, die einen Luftüberschuss-Koeffizienten zwischen 0,98 und 1,25 aufweist, bevor er in einen Industrieofen, der eine adiabatische Brennkammer (1) umfasst, eintritt;
2) Ausstoßen der in 1) vorgemischten strömenden Staubwolke über eine Brennstoffdüse (11) entlang einer tangentialen Richtung in die adiabatische Brennkammer (1), wobei die adiabatische Brennkammer (1) ein abgedichteter Wärmespeicherraum ist und die Seitenwand (2) aus einer Isoliermaterialschicht besteht; Einstellen einer volumetrischen Verbrennungsintensität der adiabatischen Brennkammer (1) auf zwischen 150 kg und 350 kg des Biomassebrennstoffs pro Kubikmeter der adiabatischen Brennkammer (1); Umgeben der Seitenwand unter Verwendung eines Heizkörpers des Industrieofens und Steuern der durch die Seitenwand (2) strömenden Wärme, dass sie weniger als 10 % der Verbrennungsenergie des mikrometergroßen Biomassebrennstoffs beträgt; wobei die Brennstoffdüse (11) mindestens eine in der Anzahl ist, und eine Ausstoßgeschwindigkeit zwischen 1 m/s und 10 m/s liegt; Vervollständigen des Vergasens und Verbrennens der strömenden Staubwolke in einem Abstand zwischen dem 0.5- und 2,5-fachen des Durchmessers der Brennstoffdüse (11), um eine Verbrennungstemperatur zwischen 1.500 °C und 1.600 °C zu erhalten; Ermöglichen, dass die ausgestoßene Flamme den Heizkörper erwärmt; und
3) Hinzufügen von Dampf in die adiabatische Brennkammer (1) während der Verbrennung, wobei das Gewichtsverhältnis von dem Dampf zu dem mikrometergroßen Biomassebrennstoff zwischen 1:30 und 1:150 liegt, um die Vergasung und Zersetzung von Zwischenprodukten zu beschleunigen, die Teer und Kohlenstoffpartikel umfassen, welche während der Verbrennung vor dem Verlassen der Flamme erzeugt wurden; Austragen von geschmolzenem Ascheanteil in Form von Flüssigglas an einem unteren Teil der adiabatischen Brennkammer (1), nachdem der geschmolzene Ascheanteil sich von der Flamme abtrennt, wenn die Verbrennung abgeschlossen ist.

2. Verfahren nach Anspruch 1, **dadurch gekennzeichnet, dass** der mikrometergroße Biomassebrennstoff mehr als 35 Gew.-% der Pulver umfasst, die eine Partikelgröße kleiner als 50 µm aufweisen; der mikrometergroße Biomassebrennstoff mehr als 75 Gew.-% der Pulver umfasst, die eine Partikelgröße kleiner als 100 µm aufweisen; und der mikrometergroße Biomassebrennstoff mehr als 90 Gew.-% der Pulver umfasst, die eine Partikelgröße kleiner als 250 µm aufweisen.

3. Verfahren nach Anspruch 1, **dadurch gekennzeichnet, dass** der mikrometergroße Biomassebrennstoff in einem Behälter unnachgiebig oder flexibel versiegelt ist, und verladen und transportiert wird und ein Volumen des Behälters zwischen 1,5 m³ und 90 m³ liegt.

4. Verfahren nach Anspruch 1 oder 2, **dadurch gekennzeichnet, dass** in 1) der Luftüberschuss-Koeffizient zwischen 1,0 und 1,15 liegt.

5. Verfahren nach Anspruch 1, 2 oder 3, **dadurch gekennzeichnet, dass** in 2) die volumetrische Verbrennungsintensität der adiabatischen Brennkammer (1) zwischen 200 kg und 300 kg des Biomassebrennstoffs pro Kubikmeter der adiabatischen Brennkammer (1) liegt und die durch die Seitenwand (2) strömende Wärme nicht mehr als 3 % bis 6 % der Verbrennungsenergie des mikrometergroßen Biomassebrennstoffs beträgt.

6. Verfahren nach Anspruch 5, **dadurch gekennzeichnet, dass** in 2) die adiabatische Brennkammer (1) der abgedichtete Wärmespeicherraum ist, der die Seitenwand (2) umfasst, die aus einer Isoliermaterialschicht aus anorganischer Faser und feuerfestem Material hergestellt wurde, und eine Dicke der Seitenwand (2) zwischen 80 mm und 320 mm liegt; und eine Höhe der adiabatischen Brennkammer (1) zwischen dem 0,8- und dem 4-fachen von dem Durchmesser der adiabatischen Brennkammer (1) liegt.

7. Verfahren nach Anspruch 5, **dadurch gekennzeichnet, dass** in 3) das Gewichtsverhältnis des Dampfes zu dem mikrometergroßen Biomassebrennstoff zwischen 1:60 und 1:120 liegt.

8. Verfahren nach einem der Ansprüche 1 bis 7, **dadurch gekennzeichnet, dass** der Industrieofen ein Kessel oder ein Ofen ist, der aus Zement, Glas oder Keramik hergestellt wurde.

## Revendications

1. Procédé de combustion nette de combustible de taille micrométrique à base de biomasse (BMF) dans une condition adiabatique, le procédé comprenant le broyage de la matière première de biomasse composée de fibre végétale en poudres solides de combustible de taille micrométrique à base de biomasse, une taille moyenne des particules des poudres solides étant inférieure à 400 µm ; et l'encapsulation hermétique du combustible de taille micrométrique à base de biomasse ; **caractérisé en ce que** le procédé comprend en outre :
1) le prémélange du combustible de taille micrométrique à base de biomasse pour former un nuage de poussière fluant ayant un coefficient d'excès d'air de 0,98 à 1,25, avant son entrée dans une étuve industrielle comprenant une chambre de combustion adiabatique (1) ;
2) l'éjection du nuage de poussière fluant prémélangé en 1) vers la chambre de combustion adiabatique (1) via une buse à combustible (11) dans une direction tangentielle, la chambre de combustion adiabatique (1) étant un espace de stockage de chaleur étanche et la paroi latérale (2) étant formée à partir d'une couche de matériau isolant ; la définition d'une intensité de combustion volumétrique de la chambre de combustion adiabatique (1) pour qu'elle soit entre 150 kg et 350 kg du combustible à base de biomasse par mètre cube de la chambre de combustion adiabatique (1) ; le fait d'entourer la paroi latérale en utilisant un corps chauffant de l'étuve industrielle, et la régulation de la chaleur s'écoulant à travers la paroi latérale (2) pour qu'elle soit inférieure à 10 % de l'énergie de combustion du combustible de taille micrométrique à base de biomasse ; la buse à combustible (11) étant au moins au nombre de 1, et une vitesse d'éjection étant comprise entre 1 m/s et 10 m/s ; la réalisation de la gazéification et la combustion du nuage de poussière fluant à une distance comprise entre 0,5 et 2,5 fois le diamètre de la buse à combustible (11) pour obtenir une température de combustion comprise entre 1 500 °C et 1 600 °C ; le fait de permettre à une flamme extrusive de chauffer le corps chauffant ; et
3) l'ajout de vapeur dans la chambre de combustion adiabatique (1) durant la combustion, et un rapport en poids de la vapeur sur le combustible de taille micrométrique à base de biomasse étant entre 1/30 et 1/150 pour accélérer la gazéification et la décomposition des intermédiaires comprenant des particules de goudron et de carbone produites durant la combustion avant de s'éloigner de la flamme ; la décharge du contenu de cendres fondues sous la forme d'un verre liquide au niveau d'une partie inférieure de la chambre de combustion adiabatique (1) après que le contenu de cendres fondues s'éloigne de la flamme lorsque la combustion est terminée.

2. Procédé selon la revendication 1, **caractérisé en ce que** le combustible de taille micrométrique à base de biomasse comprend plus de 35 % en poids de poudres ayant une taille de particules inférieure à 50 µm ; le combustible de taille micrométrique à base de biomasse comprend plus de 75 % en poids de poudres ayant une taille de particules inférieure à 100 µm ; et le combustible de taille micrométrique à base de biomasse comprend plus de 90 % en poids de poudres ayant une taille de particules inférieure à 250 µm.

3. Procédé selon la revendication 1, **caractérisé en ce que** le combustible de taille micrométrique à base de biomasse est scellé de façon rigide ou flexible dans un conteneur, et est chargé et transporté, et un volume du conteneur est entre 1,5 m³ et 90 m³.

4. Procédé selon la revendication 1 ou 2, **caractérisé en ce qu'**en 1), le coefficient d'excès d'air est compris entre 1,0 et 1,15.

5. Procédé selon la revendication 1, 2, ou 3, **caractérisé en ce qu'**en 2), l'intensité de combustion volumétrique de la chambre de combustion adiabatique (1) est entre 200 kg et 300 kg du combustible à base de biomasse par mètre cube de la chambre de combustion adiabatique (1), et la chaleur s'écoulant à travers la paroi latérale (2) n'est pas supérieure à 3 % à 6 % de l'énergie de combustion du combustible de taille micrométrique à base de biomasse.

6. Procédé selon la revendication 5, **caractérisé en ce qu'**en 2), la chambre de combustion adiabatique (1) est l'espace de stockage de chaleur étanche comprenant la paroi latérale (2) formée par une couche de matériau isolant en fibre inorganique et matériau réfractaire, et une épaisseur de la paroi latérale (2) est comprise entre 80 mm et 320 mm ; et une hauteur de la chambre de combustion adiabatique (1) est entre 0,8 et 4 fois le diamètre de la chambre de combustion adiabatique (1).

7. Procédé selon la revendication 5, **caractérisé en ce que** 3), le rapport en poids de la vapeur sur le combustible de taille micrométrique à base de biomasse est entre 1/60 et 1/120.

8. Procédé selon l'une quelconque des revendications 1 à 7, **caractérisé en ce que** l'étuve industrielle est une chaudière, ou une étuve en ciment, verre, ou céramique.
